

April 18, 1933.

A. VON ZEERLEDER

1,904,107

ELECTROPLATING WITH ALUMINUM

Filed Aug. 12, 1930



INVENTOR:

Alfred von Zeerleder

BY

Morrison, Kennedy & Campbell,  
ATTORNEYS.

## UNITED STATES PATENT OFFICE

ALFRED VON ZEERLEDER, OF NEUHAUSEN, SWITZERLAND, ASSIGNOR TO ALUMINIUM INDUSTRIE AKTIENGESELLSCHAFT, OF NEUHAUSEN, SWITZERLAND, A JOINT-STOCK COMPANY OF SWITZERLAND

## ELECTROPLATING WITH ALUMINUM

Application filed August 12, 1930, Serial No. 474,741, and in Germany August 24, 1929.

This invention relates to electroplating with aluminum, and includes both a novel process of coating metals with substantially pure aluminum and the resulting product. 5 The particular utility of the invention is in the forming of an integral aluminum coating upon iron or other ferrous or base metal, but the invention is applicable to the coating of other metals, including aluminum alloys 10 et cetera.

The main object of the invention is to afford a coated product which combines the properties or advantages of the two metals, for example the mechanical properties or 15 strength of the iron or steel on which the aluminum is deposited as a base, together with the chemical resistance of the substantially pure aluminum coating and its ability to resist corrosion. The commercial utility 20 of the invention covers a very wide field, and may be employed for example for any apparatus or mechanical part in which strength or other physical properties are essential, and which it is desirable to protect 25 from rusting or other corrosion.

Heretofore it has been attempted to coat iron or other base metal with aluminum, one method having been the rolling and welding of a thin sheet of aluminum upon the base 30 metal object, and another method having been the casting of molten aluminum around the base metal article, or casting the base metal article within a mold previously lined with sheet aluminum. These known methods 35 have never proved satisfactory as the coating is not perfect mechanically and is known to be liable to be split off or become detached if the article is bent or otherwise distorted or subjected to mechanical strain. 40 These defects are due to the lack of integral adherence between the base metal and the coating, doubtless because of the formation of a layer of oxide upon one or both of the surfaces to be united thus destroying perfect molecular union. 45

A further object of the present invention therefore is to afford a process and product overcoming the objections to the known methods, as well as to avoid the time and expense incurred in the preliminary manu-

facture of sheets or shaped layers of substantially pure aluminum. Methods have also been attempted for electroplating aluminum upon a base metal, but without practical success so far as is known, this being believed 55 to be due to the inability of such methods to deposit an adherent and dense coating, as is essential, the product having been commercially unavailable due to the formation of deposits of spongy character or in the 60 form of needles of aluminum; which shortcomings are avoided by the present invention, which affords a coating that is dense and so adherent as not to detach or split off even when the coated object, sheet, bar, 65 et cetera is subject to rolling or other working.

Other and further objects and advantages of the present invention will be explained in the hereinafter following description of an 70 illustrative embodiment thereof, or will be understood to those skilled in the subject. To the attainment of such objects and advantages the present invention consists in the novel process of electroplating with aluminum, and the novel product thereof, as well as the novel steps, operations and details, herein illustrated or described.

The present invention may be described in one aspect as consisting in the novel process 80 of electroplating with aluminum which comprises maintaining an electrolytic bath of molten salt, including a salt of aluminum, and such bath having a melting point lower than that of metallic aluminum, there being 85 immersed in the bath a solid anode of metal containing aluminum, and the object to be coated being the cathode, while passing through the bath from anode to cathode an electrolytic current so as to cause a deposition of substantially pure metallic aluminum upon the object, while the bath is replenished from the metal of the anode. More specifically the process is one for electroplating metallic objects composed of iron, or light 90 metal alloys, or other metals, with an adherent dense coating of aluminum, and the process being so carried out that not only is aluminum caused to be deposited, but supplementally thereto very small quantities of an 95 100

auxiliary metal, other than aluminum, such as lead, acting as a densifying agent and causing the deposit to be in an adherent dense form of coating. The current may be applied in such manner as to develop also the heat necessary to maintain the molten condition of the electrolyte, and for the best results the density of the current in the cathode should be substantially not higher than 10 amperes per square foot, and preferably much lower. Having thus outlined the general character of the improved process, the details of a particular embodiment thereof may be described as follows.

15 As already indicated the present process is in general an electrolytic deposition from a bath composed of suitable molten salt or salts, including a salt or salts of aluminum, the anode being a solid piece of metal containing aluminum, and the cathode being the object, article or piece to be coated which may be a sheet, bar or other shape requiring further working, or a casting or finished mechanical object such as certain parts of 25 engines.

With the present invention density and close adherence are obtained or enhanced by employing a densifying agent and causing it to cooperate in the process. This agent 30 preferably consists of a small quantity of an auxiliary metal caused to be deposited upon the cathode along with the deposit of aluminum. Practical demonstrations have established that in this way the production of 35 spongy or needle-like coatings is avoided and the deposition is rendered exceedingly dense and adherent. The auxiliary metal is preferably a selected metal, more electronegative than aluminum, and chosen for its cooperative 40 qualities, or there may be small percentages of more than one other metal. For this purpose lead is found to be advantageous, although other metals with similar quality are available.

45 It may be stated that certain ingredients which are invariably present in commercial aluminum, such as iron, carbon and sodium, and very small quantities of which tend to impair seriously the resistance of aluminum to corrosion, can nevertheless be allowed to exist in the anode in the present process, since they will be retained in the anode and selectively excluded in the electrolytic process. For this reason the aluminum coating 55 itself as deposited at the cathode is superior to the metal of the anode in the matter of resistance to corrosion. An anode therefore may be employed consisting either of raw aluminum or of aluminum alloys such for 60 example as are produced by commercial electrothermic reduction.

As an electrolyte having a lower melting point than aluminum, for the purposes of the present invention, there may be employed 65 halogen salts of aluminum mixed with halo-

gen salts of the alkaline metals, or of the alkaline earth metals, or of both such kinds of metals, under the principles set forth in U. S. Patent No. 1,709,759, granted April 16, 1929, and relating to a process of commercial production or manufacture of highly pure aluminum by electrolytic refining of less pure aluminum. 70

The additional or densifying metal of the present invention can be introduced into the process in different ways. For example it can be added to the electrolyte in the form of a suitable compound or salt of the selected metal or metals. On the other hand special auxiliary or additional anodes may be prepared and maintained in the bath containing the metal or metals to be added. In the case of providing a special separate anode for supplying the additional metal the rate at which the latter passes into the electrolyte and is deposited on the cathode may readily be regulated simply by regulating the tension or intensity at such special anode of the auxiliary current passed therethrough. 75

In regard to the quantity or percentage of the auxiliary or densifying metal which is to be added and caused to deposit for the purposes of the present invention, this depends upon the nature of the additional metal, and it can readily be determined once for all by simple tests as to each metal. In the case of lead it is found that a few tenths of one percent are sufficient to give the desired results. In general the smallest practical quantity of auxiliary metal should be employed that will avoid spongy and needle-like deposits of aluminum, and afford dense and adherent coatings. 90 95

As another factor in perfecting the results of the present process, it is found that the quality of the coating is aided by employing current densities at the cathode as low as ten amperes per square foot, or even less. 100 105

The adherence of the coating to the object or cathode will be substantially increased by the following preliminary treatment. Before the commencement of the electro-deposition the circuits may be first reversed so that the object to be coated becomes an anode, this being carried on for a short time and operating to prepare and improve the surface to receive subsequently the aluminum deposit. It is further desirable to clean preliminarily the cathode by brushing or by etching or other treatments known in the art of electro-plating. 110 115 120

The present invention is available for coating with aluminum in a simple and economical manner completed objects or mechanical pieces that are not to be submitted to further working or rolling, as for example castings of iron or other metal. In such cases the coating can be given a better appearance by subsequent polishing. Ingots, bars, sheets and the like can be coated by the present 125 130

process and thereafter submitted to further working or rolling without causing the splitting off of the coating. The present process has a special importance in regard to the 5 coating of various products whose manufacture makes it difficult or impossible to provide them with a welded coating before they have been given their final definite shape, as for instance, castings extruded sections of 10 light metals and the like.

The products of the present invention include any objects, such as those referred to, composed of iron or any other metal and carrying an electrodeposited coating of substantially 15 pure aluminum, with density of deposit and strength of adherence, and preferably with a very small percentage of a metal, more electronegative than aluminum instrumental in affording the qualities mentioned. 20

The accompanying drawing illustrates a typical mode of carrying out the invention. The vessel or cell 1 contains the molten salt electrolyte or bath 2, in which are immersed 25 one or more anodes 3 of solid metal containing aluminum. The cathode 4, which may be any metallic object or part, and is shown as an engine head casting, is held and suspended in the bath by any sort of holder or 30 clamp 5. Conductors 6 and 7 come from a direct current source, as indicated, and lead respectively to the anodes and cathodes. The bath temperature will be maintained by external heating means at a point below the 35 melting points of aluminum and of the electrodes but above the melting point of the salt mixture constituting the bath.

There have thus been described a novel process of electroplating metals, and the resulting product, embodying the principles and attaining the objects of the present invention. Since certain matters of process, product, step operation and detail may be variously modified without departing from 45 the principles of the invention it is not intended to limit the invention to such matters except to the extent set forth in the appended claims.

What is claimed is:

50 1. The process of electroplating metals, such as iron, light metal alloys, etc., with an adherent dense coating of aluminum, wherein the object to be coated is the cathode and the anode is metallic aluminum, or an alloy or mixture thereof; comprising using an electrolyte composed of a molten salt or salts, having a melting point lower than that of aluminum, and electrolytically causing aluminum together with small quantities of an auxiliary metal, comprising lead, to be deposited from the electrolyte upon the cathode. 60

65 2. The process as in claim 1, and wherein the auxiliary metal deposited in small quan-

tities with the aluminum consists wholly of lead.

3. The process as in claim 1 and wherein the density of electrolytic current at the cathode is maintained not higher than ten amperes per square foot. 70

4. The process as in claim 1 and wherein the object to be coated is connected for a short period of time as anode prior to being connected as cathode for the electroplating process for electrolytic action. 75

5. The process of electroplating with aluminum comprising maintaining an electrolytic bath of molten salt including a salt of aluminum and having a melting point lower than that of metallic aluminum, with an anode of solid metal containing aluminum and with the object to be coated as cathode therein, and introducing into the process an auxiliary agent containing lead for densifying the deposit. 80

6. The process of electroplating with aluminum comprising maintaining an electrolytic bath of molten salts including a salt of aluminum and having a melting point lower than that of metallic aluminum, with an anode of solid metal containing aluminum and with the object to be coated as cathode therein, and including with the bath or auxiliary anode a small proportion of lead tending to densify the deposit without impairing its properties. 90

7. The process as in claim 6 and wherein the lead is caused to be deposited in a proportion of less than one percent of the total deposit. 100

8. The process of electroplating aluminum upon a base metal object to afford resistance to corrosion, comprising maintaining an electrolytic bath of molten salt including a salt of aluminum and having a melting point lower than that of metallic aluminum, with an anode of solid metal containing aluminum and with the object to be coated as cathode therein, and with a separate anode containing lead as a densifying metal, not impairing the resistance to corrosion of the product, and passing currents from the anodes to the cathodes, so proportioned that only a very small percentage of the densifying metal is incorporated in the deposited coating, to give density and adherence. 105

9. An article of manufacture consisting of a metallic base and an electroplated coating thereon comprising substantially pure aluminum of strong adherence and density and such coating containing a very small percentage of lead. 110

In testimony whereof, this specification has been duly signed by. 120

ALFRED VON ZEERLEDER. 125